# EUROPEAN PATENT SPECIFICATION

(11) **EP 4 202 095 B1**
(45) Date of publication and mention of the grant of the patent: **04.02.2026**
(21) Application number: 22212748.2
(22) Date of filing: 12.12.2022
(51) Int. Cl.: D02G 3/36, D02G 3/44

(54) **YARN**
GARN
FIL

(30) Priority: 15.12.2021 FI 20216278
(43) Date of publication of application: 28.06.2023
(73) Proprietor: Valmet Technologies, Inc., 02150 Espoo (FI)
(72) Inventor: MIKKONEN, Kati, 02150 Espoo (FI); HAGFORS, Satu, 02150 Espoo (FI)
(74) Representative: Laine IP Oy

(56) References cited:
- CN-A- 113 355 779
- US-A- 4 093 512
- US-A- 5 514 438
- US-A1- 2014 096 928
- US-A1- 2017 175 301

## Description

### FIELD

The present invention relates to yarns, in particularly yarns used for manufacturing press felts.

### BACKGROUND

Generally, press felts are made from yarns consisting of monofilaments or twisted monofilaments. In some special types also spun yarn is used together with the monofilaments, either twisted or wound around the filaments. The purpose of the spun yarn is to densify the felt and create a fast start-up and good nip dewatering.

US5514438 A1 discloses a papermakers fabric comprising a felt made up of a base cloth and a batt of fibres needled to the base cloth. The papermakers fabric is woven from machine direction yarns and cross machine direction yarns. The machine direction yarns comprise a core of cabled monofilaments surrounded by a sheath of multifilaments.

US4093512 A discloses papermakers' belts for use in papermaking machines which belts comprise ultra-high modulus load bearing yarn comprised of poly(para-phenylene terephthalamide).

US20140096928 A1 discloses a paper machine belt, wherein some of the threads or all of the threads being made partially or entirely of a bioplastic.

US20170175301 A1 discloses a hybrid cord comprising a first yarn, without initial S or Z twist, of continuous polymeric filaments forming the core of the cord, the yarn being a non-bulked yarn, and a second yarn, without initial S or Z twist, of continuous polymeric filaments, the second yarn being a bulked yarn that is wrapped around the first yarn.

CN113355779 A discloses a covering yarn comprising a central tow and covering filaments wound on the central tow. The central tow comprises one or two or more central filaments. The central filaments are selected from synthetic fibers and the covering filaments are selected from plant fibers or mixed fibers.

However, when the spun yarn is used in a woven press felt, it causes a lot of dusting during weaving the press felt. So, there is a need to improve composition of the yarns. Furthermore, in view of the increasing requirements for sustainability and decreasing the amount of microplastics emitted to nature together with emerging interest to reduce fossil-based raw materials, there is also a need for novel yarns that exceed these expectations without sacrificing their mechanical performance.

### SUMMARY OF THE INVENTION

According to a first aspect of the present invention, there is provided a yarn comprising a plurality of monofilaments twisted together, and a multifilament wound around the plurality of monofilaments, wherein the multifilament comprises a bio-based material.

According to a second aspect of the present invention, there is provided an industrial textile comprising the yarn.

According to a third aspect of the present invention, the yarn is used in an industrial textile, such as a press felt or a filter fabric.

According to a fourth aspect of the present invention, the yarn is used in a paper machine clothing.

### BRIEF DESCRIPTION OF THE DRAWINGS

FIGURE 1 illustrates a yarn in accordance with at least some embodiments of the present invention.

### EMBODIMENTS

In the present context, the term "bio-based material" refers to a material, which is wholly or partly derived from renewable biomass sources, such as plants, trees or animals. The material can be obtained from for example, a sugar containing plant (e.g. corn or sugar cane), plant fat or oil (e.g. castor oil), organic acid (e.g. succinic acid), corn starch, straw, woodchips, sawdust, recycled food waste. The bio-based material can be obtained by processing from natural biopolymers including polysaccharides (e.g. starch, cellulose, nanocellulose, microcellulose, chitosan and alginate) and proteins (e.g. soy protein, gluten and gelatin), or by chemically synthesizing from sugar derivatives (e.g. lactic acid) and lipids (oils and fats) from either plants or animals, or biologically generated by fermentation of sugars or lipids. This kind of bio-based material can be for example, polylactic acid (PLA), bio-polyamide (bio-PA), bio-polybutylene succinate (bio-PBS), bio-polyethylene (bio-PE), bio-polyethylene terephthalate (bio-PET), bi-polypropylene (bio-PP), or bio-polyhydroxyalkanoate (bio-PHA). Cellulose-based materials are bio-based materials manufactured from cellulose, such as cellulose fibres or cellulose derivate, for example, by dissolving pulp, treating pulp mechanically or transforming pulp directly to fibres with water and without any chemicals. The cellulose-based material can be for example, viscose, lyocell, cupro, acetate, modal, or cellulose carbamate.

In the present context, the term "synthetic material" refers to synthetic man-made polymers, which are derived from crude oil. The synthetic material can be for example, polyamide (PA), polyester (PET), polyethylene naphthalate (PEN) or polyphenylene sulphide (PPS).

In the present context, the term "overfeed" means that a multifilament yarn is fed faster than monofilaments in a yarn manufacturing. So, a length of the multifilament is longer than a length of the monofilament in the yarn.

Generally used yarns consisting twisted monofilaments and a spun yarn wound around the monofilaments cause a lot of dusting during weaving of the press felt. Furthermore, there is a need for sustainable yarns having a low carbon footprint. It is also important to decrease the amount of microplastics emitted from the press felt during the use.

A yarn 100 comprises a plurality of monofilaments 101, 102, 103, 104 twisted together, and a multifilament 105 wound around the plurality of monofilaments 101, 102, 103, 104. The multifilament 105 comprises a bio-based material. It has surprisingly been found that the whole yarn does not have to be made from high quality materials, such as synthetic polyamide, but a part of the yarns, i.e. the multifilament, can be made from a material, which has a lower strength. When the material wears off due to its lower mechanical strength or dissolves due to its chemical composition, it opens the felt structure preventing it from getting too dense. A core comprising monofilaments provides strength for the yarn, and the multifilament around the core provides a densifying effect that is needed at the start-up of the felt. Therefore, the multifilament can be made of materials having a lower carbon footprint. Thanks to this, a carbon footprint of the whole yarn and products made from the yarn is reduced. So, the yarn comprising a bio-based material provides more sustainable option for generally used yarns manufactured entirely from fossil-based raw materials. So, the yarn provides longer life time for the press felt by keeping it open longer and a low carbon footprint without sacrificing mechanical properties of the yarn.

According to an embodiment, the bio-based material is a cellulose-based material. Cellulose is natural, biodegradable and recyclable material and causes significantly smaller carbon dioxide emissions than synthetic materials. Therefore, the cellulose-based material is a more sustainable choice than fossil-based materials, which are refined and processed from crude oil.

According to an embodiment, the cellulose-based material is selected from the group of viscose, lyocell, cupro, acetate, modal and cellulose carbamate. A utilization of wood-based cellulose as the raw material for fibres leads to a carbon-neutral cycle, whereby carbon dioxide, which binds to wood, is transported with the product and decomposes back into the atmosphere as a result of burning or biodegradation. Further, production of the cellulose fibres has lower impact on land use and lower emissions than production of many other fibers, such as cotton, allowing more farmland to be used for food production.

According to an embodiment, the bio-based material is selected from the group of polylactic acid (PLA), bio-polyamide 6.10, bio-polyamide 4.10, bio-polyamide 5.10, bio-polyamide 10, bio-polyamide 10.10, bio-polyamide 11, bio-polybutylene succinate (bio-PBS), bio-polyethylene (bio-PE), bio-polyethylene terephthalate (bio-PET), bio-polypropylene (bio-PP), or bio-polyhydroxyalkanoate (bio-PHA). PLA can be manufactured from fermented plant starch, such as from corn, cassava, sugarcane or sugar beet pulp. Bio-polyamides and other bio-polymers are more sustainable choices than fossil-based polyamides, which are refined and processed from crude oil.

The bio-based material can be also biodegradable. For example, PLA, bio-PBS, bio-PP and bio-PHA are also biodegradable. Thus, these materials are capable of being decomposed by bacteria or other living organisms and thereby avoiding pollution.

According to an embodiment, the plurality of monofilaments 101, 102, 103, 104 comprises polyamide (PA). The polyamide can be bio-based polyamide (bio-PA). Bio-based polyamide can be for example, bio-polyamide 6.10, bio-polyamide 4.10, bio-polyamide 5.10, bio-polyamide 10, bio-polyamide 10.10, or bio-polyamide 11. The above-mentioned polyamides are excellent choices when mechanical strength and wear resistance is needed. Polyamide 6 fibres are tough, possessing high tensile strength and elasticity. They are highly resistant to abrasion and chemicals, such as alkalis. Polyamide 6 has high water absorption. Polyamide 6.6 has a high mechanical strength, a rigidity and a good heat and chemical stability. Polyamide 6.10 has high impact resistance, chemical resistance and retention of dimension. Polyamide 11 has lower values of density, flexural and Young's modulus, water absorption, as well as melting and glass transition temperatures than polyamide 6. However, polyamide 11 is seen to have increased elasticity, abrasion resistance and, due to lower water absorption, dimensional stability in the presence of moisture than polyamide 6.

According to an embodiment, the yarn 100 comprises 3-24 monofilaments 101, 102, 103, 104, preferably 3-12 monofilaments 101, 102, 103, 104, more preferably 3-6 monofilaments 101, 102, 103, 104. For example, the yarn 100 can comprise 4, 6, 8 or 9 monofilaments 101, 102, 103, 104.

According to an embodiment, a twist direction of the plurality of monofilaments 101, 102, 103, 104 is the same as a twist direction of the multifilament 105. The direction of the twist may be to the right (Z twist), or to the left (S twist).

Alternatively, a twist direction of the plurality of monofilaments 101, 102, 103, 104 is the opposite as a twist direction of the multifilament 105. The direction of the twist may be to the right (Z twist), or to the left (S twist).

FIGURE 1 illustrates a yarn 100 in accordance with at least some embodiments. The yarn comprises four monofilaments 101, 102, 103, 104 and a multifilament 105 wound around the said monofilaments. A twist direction of the four monofilaments 101, 102, 103, 104 is the same as a twist direction of the multifilament, being a left twist.

According to an embodiment, diameters of the plurality of the monofilaments 101, 102, 103, 104 are 0.1-0.6 mm, preferably 0.2 mm. The diameters of the monofilaments can be selected according to the intended use of the yarn and the number of the monofilaments. For example, when the number of the monofilaments is increased, the diameter of the monofilaments can be decreased.

According to an embodiment, the multifilament 105 has a linear density of 50-150 dtex.

The multifilament is twisted. Twisting of the multifilament 105 facilitates its handling and entangles filaments of the multifilament together. Further, the twisted multifilament has higher strength and elasticity (i.e. higher stretch). A surface of the twisted multifilament does not wear out so easily. Further, twisting can be used for forming texture to the yarn.

When the multifilament 105 is twisted, it may be twisted in a first direction. Then, the multifilament 105 may be twisted in a second direction, which is opposite direction than the first direction, around the plurality of monofilaments 101, 102, 103, 104. Twisting of the multifilament provides a good tenacity.

The multifilament 105 can be also textured. Texturing can be provided by curling the multifilament.

The yarn 100 has an overfeed of the multifilament 105 of 5-25 %, preferably about 15 %. The overfeed provides a densifying effect that is needed at the start-up of the felt.

The cross-section of the monofilaments or the multifilament 105 can be round, square, rectangular, oval or any other suitable shape.

According to an embodiment, a linear density of the yarn 100 is 200-600 tex.

In an embodiment not covered by the subject-matter of the claims, a method for manufacturing a yarn 100 comprises providing a plurality of monofilaments 101, 102, 103, 104 and a multifilament 105, twisting the plurality of the monofilaments together, and simultaneously or afterwards, winding the multifilament 105 around the plurality of the monofilaments 101, 102, 103, 104. The multifilament comprises a bio-based material. So, twisting the plurality of the monofilaments together can be done first. After that, the multifilament 105 can be wound around the plurality of the monofilaments. Alternatively, twisting the plurality of the monofilaments together and winding the multifilament 105 around the plurality of the monofilaments can be done simultaneously.

According to an embodiment, an industrial textile can comprise the yarn 100 according to an above-mentioned embodiment. The yarn provides fast start-up and good nip dewatering for press felts made from it. When the yarn comprises the multifilament, there is also less dusting when weaving textiles from the yarn. In addition, when the bio-based multifilament is wearing off, it opens the felt structure thus lengthening its lifetime.

The yarn 100 can be used in an industrial textile, such as a press felt or a filter fabric. The industrial textile can be woven or non-woven.

The yarn 100 can be used in a paper machine clothing.

It is to be understood that the embodiments of the invention disclosed are not limited to the particular structures, process steps, or materials disclosed herein, but are extended to equivalents thereof as would be recognized by those ordinarily skilled in the relevant arts. It should also be understood that terminology employed herein is used for the purpose of describing particular embodiments only and is not intended to be limiting.

While the forgoing examples are illustrative of the principles of the present invention in one or more particular applications, it will be apparent to those of ordinary skill in the art that numerous modifications in form, usage and details of implementation can be made without the exercise of inventive faculty, and without departing from the principles and concepts of the invention. Accordingly, it is not intended that the invention be limited, except as by the claims set forth below.

### REFERENCE SIGNS LIST

- 100: yarn
- 101-104: monofilament
- 105: multifilament

## Claims

1. A yarn (100) comprising:
- a plurality of monofilaments (101 102, 103, 104) twisted together, and
- a multifilament (105) wound around the plurality of monofilaments (101, 102, 103, 104),
**characterised in that** the multifilament (105) comprises a bio-based material, the yarn (100) has an overfeed of the multifilament (105) of 5-25 %, and the multifilament (105) is twisted.

2. The yarn (100) of claim 1, wherein the plurality of monofilaments (101, 102, 103, 104) comprises a bio-based polyamide, such as bio-polyamide 6.10, bio-polyamide 4.10, bio-polyamide 10, bio-polyamide 10.10 or bio-polyamide 11, or a synthetic polyamide or a recycled polyamide, such as polyamide 6, polyamide 6.6 or polyamide 12.

3. The yarn (100) of any one of the preceding claims, comprising 3-24 monofilaments (101, 102, 103, 104), preferably 3-12 monofilaments (101, 102, 103, 104), more preferably 3-6 monofilaments (101, 102, 103, 104).

4. The yarn (100) of any one of the preceding claims, wherein the bio-based material is a cellulose-based material.

5. The yarn (100) of claim 4, wherein the cellulose-based material is selected from the group of viscose, lyocell, cupro, acetate, modal and cellulose carbamate.

6. The yarn (100) of any one of the preceding claims 1-3, wherein the bio-based material is selected from the group of polylactic acid, bio-polyamide 6.10, bio-polyamide 4.10, bio-polyamide 5.10, bio-polyamide 10, bio-polyamide 10.10, bio-polyamide 11, bio-polybutylene succinate, bio-polyethylene, bio-polyethylene terephthalate, bio-polypropylene, bio-polyhydroxyalkanoate.

7. The yarn (100) of any one of the preceding claims, wherein a twist direction of the plurality of monofilaments (101, 102, 103, 104) is the same as a twist direction of the multifilament (105).

8. The yarn (100) of any one of the preceding claims, wherein diameters of the plurality of monofilaments (101, 102, 103, 104) are 0.1-0.6 mm, preferably 0.2 mm.

9. The yarn (100) of any one of the preceding claims, wherein the multifilament yarn (105) has a linear density of 50-150 dtex.

10. The yarn (100) of any one of the preceding claims, having an overfeed of the multifilament (105) of about 15 %.

11. The yarn (100) of any one of the preceding claims, having a linear density of 200-600 tex.

12. An industrial textile comprising a yarn (100) of any one of claims 1 to 11.

13. Use of a yarn (100) of any one of the claims 1 to 11 in an industrial textile, such as a press felt or a filter fabric.

14. Use of a yarn (100) of any one of the claims 1 to 11 in a paper machine clothing.

## Patentansprüche

1. Garn (100), umfassend:
- eine Vielzahl von Monofilamenten (101 102, 103, 104), die miteinander verdrillt sind, und
- ein Multifilament (105), das um die Vielzahl von Monofilamenten (101, 102, 103, 104) gewickelt ist,
**dadurch gekennzeichnet, dass** das Multifilament (105) ein biobasiertes Material umfasst, das Garn (100) eine Voreilung des Multifilaments (105) von 5-25 % aufweist und das Multifilament (105) verdrillt ist.

2. Garn (100) nach Anspruch 1, wobei die Vielzahl von Monofilamenten (101, 102, 103, 104) ein biobasiertes Polyamid, wie etwa Bio-Polyamid 6.10, Bio-Polyamid 4.10, Bio-Polyamid 10, Bio-Polyamid 10.10 oder Bio-Polyamid 11 oder ein synthetisches Polyamid oder ein recyceltes Polyamid, wie etwa Polyamid 6, Polyamid 6.6 oder Polyamid 12, umfasst.

3. Garn (100) nach einem der vorstehenden Ansprüche, umfassend 3-24 Monofilamente (101, 102, 103, 104), bevorzugt 3-12 Monofilamente (101, 102, 103, 104), besonders bevorzugt 3-6 Monofilamente (101, 102, 103, 104).

4. Garn (100) nach einem der vorstehenden Ansprüche, wobei das biobasierte Material ein Material auf Zellulosebasis ist.

5. Garn (100) nach Anspruch 4, wobei das Material auf Cellulosebasis aus der Gruppe ausgewählt ist, die aus Folgendem besteht: Viskose, Lyocell, Cupro, Acetat, Modal und Cellulosecarbamat.

6. Garn (100) nach einem der vorstehenden Ansprüche 1-3, wobei das biobasierte Material aus der Gruppe ausgewählt ist, die aus Folgendem besteht: Polylactid, Bio-Polyamid 6.10, Bio-Polyamid 4.10, Bio-Polyamid 5.10, Bio-Polyamid 10, Bio-Polyamid 10.10, Bio-Polyamid 11, Bio-Polybutylensuccinat, Bio-Polyethylen, Bio-Polyethylenterephthalat, Bio-Polypropylen, Bio-Polyhydroxyalkanoat.

7. Garn (100) nach einem der vorstehenden Ansprüche, wobei eine Verdrillungsrichtung der Vielzahl von Monofilamenten (101, 102, 103, 104) mit der Verdrillungsrichtung des Multifilaments (105) übereinstimmt.

8. Garn (100) nach einem der vorstehenden Ansprüche, wobei Durchmesser der Vielzahl von Monofilamenten (101, 102, 103, 104) 0,1 bis 0,6 mm, bevorzugt 0,2 mm, betragen.

9. Garn (100) nach einem der vorstehenden Ansprüche, wobei das Multifilamentgarn (105) eine lineare Dichte von 50-150 dtex aufweist.

10. Garn (100) nach einem der vorstehenden Ansprüche, das eine Voreilung des Multifilaments (105) von etwa 15 % aufweist.

11. Garn (100) nach einem der vorstehenden Ansprüche, das eine lineare Dichte von 200-600 tex aufweist.

12. Industrielles Textil, umfassend ein Garn (100) nach einem der Ansprüche 1 bis 11.

13. Verwendung eines Garns (100) nach einem der Ansprüche 1 bis 11 in einem industriellen Textil, wie etwa einem Pressfilz oder einem Filtergewebe.

14. Verwendung eines Garns (100) nach einem der Ansprüche 1 bis 11 in einer Papiermaschinenbespannung.

## Revendications

1. Fil (100) comprenant :
- une pluralité de monofilaments (101, 102, 103, 104) torsadés ensemble, et
- un multifilament (105) enroulé autour de la pluralité de monofilaments (101, 102, 103, 104),
**caractérisé en ce que** le multifilament (105) comprend un matériau biosourcé, le fil (100) présente une suralimentation du multifilament (105) de 5-25 % et le multifilament (105) est torsadé.

2. Fil (100) selon la revendication 1, dans lequel la pluralité de monofilaments (101, 102, 103, 104) comprennent un polyamide biosourcé, tel que le bio-polyamide 6.10, le bio-polyamide 4.10, le bio-polyamide 10, le bio-polyamide 10.10 ou le bio-polyamide 11, ou un polyamide synthétique ou un polyamide recyclé, tel que le polyamide 6, le polyamide 6.6 ou le polyamide 12.

3. Fil (100) selon l'une quelconque des revendications précédentes, comprenant 3-24 monofilaments (101, 102, 103, 104), de préférence 3-12 monofilaments (101, 102, 103, 104), plus préférentiellement 3-6 monofilaments (101, 102, 103, 104).

4. Fil (100) selon l'une quelconque des revendications précédentes, dans lequel le matériau biosourcé est un matériau cellulosique.

5. Fil (100) selon la revendication 4, dans lequel le matériau cellulosique est choisi dans le groupe consistant en la viscose, le lyocell, le cupro, l'acétate, le modal et le carbamate de cellulose.

6. Fil (100) selon l'une quelconque des revendications précédentes 1-3, dans lequel le matériau biosourcé est choisi dans le groupe consistant en l'acide polylactique, le bio-polyamide 6.10, le bio-polyamide 4.10, le bio-polyamide 5.10, le bio-polyamide 10, le bio-polyamide 10.10, le bio-polyamide 11, le bio-polybutylène succinate, le bio-polyéthylène, le bio-polyéthylène téréphtalate, le bio-polypropylène, le bio-polyhydroxyalcanoate.

7. Fil (100) selon l'une quelconque des revendications précédentes, dans lequel un sens de torsion de la pluralité de monofilaments (101, 102, 103, 104) est le même qu'un sens de torsion du multifilament (105).

8. Fil (100) selon l'une quelconque des revendications précédentes, dans lequel les diamètres de la pluralité de monofilaments (101, 102, 103, 104) sont de 0,1-0,6 mm, de préférence 0,2 mm.

9. Fil (100) selon l'une quelconque des revendications précédentes, dans lequel le fil multifilament (105) présente une densité linéaire de 50-150 dtex.

10. Fil (100) selon l'une quelconque des revendications précédentes, présentant un suralimentation du multifilament (105) d'environ 15 %.

11. Fil (100) selon l'une quelconque des revendications précédentes, présentant une densité linéaire de 200-600 tex.

12. Textile industriel comprenant un fil (100) selon l'une quelconque des revendications 1 à 11.

13. Utilisation d'un fil (100) selon l'une quelconque des revendications 1 à 11 dans un textile industriel, tel qu'un feutre de presse ou un tissu filtrant.

14. Utilisation d'un fil (100) selon l'une quelconque des revendications 1 à 11 dans une toile pour machine à papier.
